

Sept. 13, 1932.

E. FALKENTHAL

1,877,569

ELECTROMAGNETIC APPARATUS

Filed Jan. 29, 1931

Fig. 1



Fig. 2



Fig. 3



INVENTOR  
Erwin Falkenthal

BY

*Samuel Detrolak*

ATTORNEY

## UNITED STATES PATENT OFFICE

ERWIN FALKENTHAL, OF BERLIN-DAHLEM, GERMANY, ASSIGNOR OF FIFTY PER CENT  
TO RADIO PATENTS CORPORATION, OF NEW YORK, N. Y., A CORPORATION OF  
NEW YORK

## ELECTROMAGNETIC APPARATUS

Application filed January 29, 1931, Serial No. 512,009, and in Germany February 19, 1930.

My invention relates to magnetic or electromagnetic apparatus and more particularly to iron cores serving as conductors for the magnetic lines of force or for increasing the amount of magnetic flux through a given surface.

The invention has for its object an iron core with improved magnetic characteristics which remain unaffected during a considerable period of time.

Another object of the invention is to provide means whereby the surface of the iron sheets, of which the core is composed in accordance with the established practice, is prevented from oxidation due to outside influences, such as of the atmospheric air.

These and further objects will become more apparent by the following detailed description, in conjunction with the accompanying drawing, which I have chosen for illustrating more clearly the novel features of the invention.

Figures 1 and 2 illustrate in a schematic manner a front and side view of a transformer having an iron core in accordance with the invention; and

Figure 3 is a fractional view of the cross section of an individual iron sheet shown in a largely magnified scale for clearness of illustration.

It is well known according to the customary practice to construct the cores for electro-magnets subjected to magnetic flux variations by assembling individual iron sheets stacked upon each other. In order to prevent losses due to hystereses, it is furthermore common to use an alloy of iron and silicium or nickel, or any other suitable alloy, in place of pure iron. Such iron sheets commonly used in construction of electrical machines and signalling apparatus have, in most cases, a very thick oxide surface due to the particular treatment during the manufacturing process, especially when the sheets have been annealed, or furthermore when they have been stored during long periods of time. This has the effect that the effective cross section of the magnetic cores composed of such sheets is considerably decreased, naturally entailing further losses as to the magnetic action.

It has already been suggested to obviate these disadvantages by galvanizing the iron or alloy sheets. This method, however, could not be used satisfactorily as yet, probably in view of the increased time and expense required for the necessary preliminary treatment of the sheets for such a process. This preliminary treatment has to be carried out very carefully, as otherwise no permanent and effective deposits on the sheets could be secured.

If, furthermore, it is desired to minimize or practically eliminate losses due to circulating or eddy currents in the iron core produced by variation of the magnetic flux passing through it, it is necessary to apply the sheets with a coating of an insulating material, such as lacquer or paper, as is usually used in practice. This latter method causes a considerable increase in the cost of the sheets, as will be obvious and in this case the effective iron cross section also receives a considerable decrease, on account of the space required for the lacquer or paper insulation.

The afore-mentioned disadvantages are overcome by the present invention herein-after described and consisting in the use of iron or suitable alloy sheets—iron silicium or iron nickel alloys, etc.—provided with a very thin surface coating of aluminum. This coating may be applied preferably according to a well-known process by rolling on to the iron sheet thin aluminum foil at normal or cold temperature and under a very high pressure. Through such an aluminum coating the surface oxidation of the iron sheets is prevented even after very extended storing periods, whereby an increase of the electric and magnetic efficiency of the apparatus comprising such sheets is obtained.

The afore-mentioned process presents the further advantage that the hystereses losses in view of the additional surface coating of the iron sheets is still further decreased to some extent. The cost of the aluminum coating which usually has a thickness of a few thousandths of a millimeter is fairly small when applied simultaneously during the rolling process of the sheets; that is, during one and the same production process. In such

cases where it is desired to decrease the eddy current losses, the aluminum coating in accordance with a further feature of the invention is furthermore provided with an oxide surface by surface oxidation in that, for instance, the sheets after leaving the rolling mills are passed through a suitable solution, such as acetic acid, whereby a very thin, non-conducting aluminum oxide surface is produced. Thus, this insulating surface can also be produced simultaneously during the rolling process of the sheets; i. e., in the same production step, saving thereby considerable time and expense as compared to the hitherto used process of applying a lacquer or paper insulation.

Iron or magnet cores as hereinbefore described and forming the subject matter of my invention may be used advantageously in any kind of magnetic or electro-magnetic apparatus, such as for field coils and as armature cores of electric machines, magnetic cores for signaling apparatus, such as of telephones, loud speakers and, in general, in all such cases where iron cores composed of individual sheets are required.

Referring to the drawing, I have illustrated in a schematic manner a transformer as used for electrical purposes, comprising a core C consisting of individual iron punchings *i* or punchings of a suitable iron alloy stacked upon each other as shown by Figure 2. The core carries a winding *w*, which is wound on a suitable support, in a manner well known in the art. The winding *w* may consist of a primary and secondary winding, or it may be a single winding, as in the case of an auto-transformer or of a choke coil and the like. The core C has the object of serving as a conductor of the magnetic lines of force or the magnetic flux, as indicated by the dotted line *f*. This flux may be a unidirectional flux varying in intensity, or may be an alternating flux periodically changing its direction and in both cases it is desired to prevent the generation of circulating or eddy currents, for which purpose the core consists of sheets *i* separated from each other by the non-conducting oxide surface of the aluminum coating applied to the sheets *i*, as seen from Figure 2, or more clearly from Figure 3. In Figure 2 the dimensions of the aluminum coating and its oxide surface *o* are unproportionately exaggerated in comparison to the iron core base *i*. Figure 3 shows approximately the real proportions in an enlarged manner.

Although I have described my invention with specific reference to the disclosure and the showing of the drawing, it is understood that modifications and variations are possible in accordance with its general aspects and broad scope, as expressed in the appended claims.

What I claim is:—

1. In an iron core for electrical apparatus composed of iron sheets provided with an aluminum coating.

2. In a magnetic core for electrical apparatus, being composed of single sheets stacked upon each other, in which iron sheets are used provided with a thin aluminum coating.

3. In a magnetic core for electrical apparatus, being composed of single sheets stacked upon each other, in which said sheets consist substantially of magnetic material with a thin aluminum coating, the outside surface of said aluminum coating, in turn, being provided with a second aluminum oxide coating.

4. In a magnetic core for electric apparatus, being composed of single sheets stacked upon each other, in which said sheets consist substantially of an iron base provided with a thin aluminum coating, the outside surface of said aluminum coating consisting of aluminum oxide.

5. In a magnetic core for electrical apparatus, comprising iron sheets of magnetic base material, the method of manufacturing said iron sheets which consists in rolling on under pressure a thin aluminum foil to the magnetic base material and subsequently passing the sheet through an oxidizing agent.

6. In a magnetic core for electrical apparatus, comprising aluminum coated sheets, the method of manufacturing said aluminum coated sheets, which consists in rolling on under pressure a thin aluminum foil to the iron sheets and subsequently passing the sheets through a bath of acetic acid for producing an aluminum oxide surface.

In testimony whereof I affix my signature.  
ERWIN FALKENTHAL.

105

110

115

120

125

130